# EUROPEAN PATENT SPECIFICATION

(11) **EP 3 031 941 B1**
(45) Date of publication and mention of the grant of the patent: **05.07.2017**
(21) Application number: 15198382.2
(22) Date of filing: 06.12.2013
(51) Int. Cl.: C22C 21/00

(54) **HEAT RESISTANT ALLOY FOR PRODUCTION OF AEROSOL CANS**
HITZEBESTÄNDIGE LEGIERUNG ZUR HERSTELLUNG VON AEROSOLDOSEN
ALLIAGE RÉSISTANT À LA CHALEUR POUR LA PRODUCTION DE BOMBES AÉROSOLS

(43) Date of publication of application: 15.06.2016
(62) Divisional of application: 13466032.3
(73) Proprietor: Moravia Cans a.s., 687 71 Bojkovice (CZ)
(72) Inventor: SEDLACEK, Jan, 69676 Louka (CZ); DIVOKY, Rudolf, 68801 Uhersky Brod (CZ); KROVINA, Jan, 687 25 Hluk (CZ); FOKSOVA, Veronika, 76326 Luhacovice (CZ)
(74) Representative: Malusek, Jiri

(56) References cited:
- EP-A2- 1 624 083
- Deutsche Norm - DIN EN 573-3: "Aluminium und Aluminiumlegierungen-Chemische Zusammensetzung und Foem von Halbzeug- Teil3: Chemiche Zusammensetzung und Erzeugnisformen; Deutsche fassung EN 573-3:2009", , 1 August 2009 (2009-08-01), pages 1-32, XP055266255, Retrieved from the Internet: URL:http://www.siblenta.ru/upload/files/DI N EN 573-3 2009-08.pdf [retrieved on 2016-04-18]

## Description

### Background of the invention

At the present time, aerosol cans are manufactured either from pure aluminium or from aluminium alloys. In the former case, 1000-series aluminium according to the European standard EN 573-3 is mostly used. The most common aluminium grades are EN AW 1050A having the minimum Al content of Al 99.5% and EN AW 1070A having the minimum Al content of 99.7%.

In the latter case, aerosol cans are mostly made of 3000-series aluminium alloys according to the European standard EN 573-3. The most common aluminium alloy grades are EN AW 3102 having the Mn content of approximately 0.3% and EN AW 3207 having the Mn content of approximately 0.6%.

For the manufacture of aerosol cans, aluminium and its alloys are mostly supplied in the form of slugs.

Such slugs are manufactured in a continuous two-phase process comprising the following steps.

### a.) Phase 1 - Manufacture of strips

- Melting down ingots in melting furnaces.
- Transfer of molten aluminium into a holding furnace.
- Continuous casting of a strip.
- Hot rolling of the cast strip.
- Cold rolling of the cast strip.
- Coiling the rolled strip.

### b.) Phase 2 - Manufacture of slugs

- Uncoiling the rolled strip.
- Punching the slugs in a blanking press.
- Annealing of the slugs.
- Cooling down of the slugs.
- Surface finishing of the slugs (tumbling, sand blasting, vibration).
- Packaging of the slugs.

The method of manufacturing aerosol cans can be described as follows:
- Applying a lubricant to the slugs.
- Backward impact extrusion.
- Wall ironing of the can.
- Brushing of the can.
- Degreasing of the can.
- Application of the inner varnish layer + curing in a polymerization oven
- Application of the basecoat + curing in oven.
- Application of the decorative inks + curing in oven.
- Application of the overcoat + curing in oven.
- Shaping the cans on the necking press.

The above described materials according to the standards EN AW 1050A and EN AW 1070A respectively exhibit significant levels of formability and work hardening which make them ideal for the manufacture of aerosol cans in a backward impact extrusion process. Aluminium alloys EN AW 3102 and EN AW 3207 offer enhanced mechanical properties (strength) and hence better rigidity and pressure resistance of finished aerosol cans. Nevertheless, the mechanical properties of these materials are changed when the cans pass through a curing oven in which polymerization of the inner varnish layer takes place. The curing (polymerization) temperatures of the inner varnish layers range between 210 and 255°C, the respective curing process lasting about 10 minutes. Under such temperatures, partial annealing of the can bodies occurs causing the mechanical strength of the same to decrease.

In order to eliminate the above undesirable effect, thicker walls of the aerosol cans must be selected which are necessary for achieving the required safety and technological specifications, particularly a sufficient pressure resistance, of the cans. This leads to an significant increase of the consumption of input materials.

In US 6,543,636 a process of making cans from aluminium alloy is presented and alloy 1050 A was chosen as the as the suitable one. This alloy is known as EN AW 1050A according to the EU norm and is broadly used. Nevertheles, for some application tensile strength (Rm) of the cans is not satisfactory enough when being subject to the higher temperature.

### Summary of the invention

The above drawbacks are eliminated by the heat-resistant alloy for the production of aerosol cans having the features defined in the characterizing part of claim 1.

### Brief description of the drawings

The invention will be further explained with reference to the accompanying drawings in which Fig. 1 shows the temperature dependences of the strengths of the new alloys in comparison with those of standard alloys by means of a graphical representation.

The subject matter of the present invention is a new, modified heat resistant aluminium based alloy provided for eliminating the effect of weakening the material of the cans passing through a curing oven. Thereby, the desired enhancement of the mechanical properties of aerosol cans is achieved in comparison with standard (conventionally used) materials, along with the reduction of the wall thickness and increase of the pressure resistance of the same. Particularly, the above favourable effect is achieved by adding an anti-recrystallization admixture formed by Zr (zirconium) for the purpose of modifying the composition of aluminium alloys falling under the EN AW 3207 standard.

The chemical compositions of the commonly used, non-modified alloys have the following limit values in accordance with EN 573-3 in percent by weight:
EN AW 3207
Si ≤ 0.30; Fe ≤ 0.45; Cu ≤ 0.10; Mn 0.40-0.80; Mg ≤ 0.10; Zn ≤ 0.10; Al remainder

The alloy according to the invention has new chemical composition with added Zr, the proportion of the new constituent ranging between 0.10 and 0.15% by weight. The addition of Zr gives rise to completely new alloy which cannot be categorized in the existing classes according to the standard EN 573-3. Therefore, the new alloys will be referred to as MC alloys hereinafter, namely MC4 (EN AW 3207 + Zr). The composition of the new alloy (in percent by weight) is as follows:
Alloy MC4
Si ≤ 0.30; Fe ≤ 0.45; Cu ≤ 0.10; Mn 0.40÷0.80; Mg ≤ 0.10; Zn ≤ 0.10; Zr = 0.05÷0.20;
Al remainder; (sum of all secondary elements ≤ 0.10)

In order to verify the anti-recrystallization effect during the aerosol can production process, the new alloys were compared with the known, commonly used materials. The outcome is graphically represented in Fig. 1 where the first standard material according to EN AW 1050A, herein specifically referred to as alloy A5, is compared with the new alloy MC1_A *which is not subject of this application.* and the second standard material according to EN AW 3102, herein specifically referred to as alloy A3Mn, is compared with the new alloy MC4_A containing the added anti-recrystallization constituent Zr. The cans, which were made of the above materials under the same technological conditions, had identical wall specifications.

The standard alloys used for comparison purposes of anti-recrystallization effect are designated as follows:
Alloy A5 (aluminium according to EN AW 1050A) having the following chemical composition in percent by weight:
   Si = 0.08; Fe = 0.24; Cu ≤ 0.005; Mn ≤ 0.005; Mg ≤ 0.005; Zn = 0.01; Ti = 0,02; Al remainder

Alloy A3Mn (aluminium alloy according to EN AW 3102) having the following chemical composition in percent by weight:
Si = 0.07; Fe = 0.25; Cu ≤ 0.005; Mn = 0.29; Mg ≤ 0.005; Zn = 0.01; Ti = 0.02; Al remainder

The newly developed alloy used for comparison purposes of anti-recrystallization effect are designated as follows:
Alloy MC4_A having the following chemical composition in percent by weight:
   Si = 0.05÷0.09; Fe = 0.23÷0.27; Cu ≤ 0.005; Mn = 0.58÷0.62; Mg ≤ 0.005; Zn ≤ 0.015; Ti = 0.01÷0.03; Zr = 0.12; Al remainder

Table 1 shows the mechanical properties of the cans made of the above materials. During the comparison, the values of the tensile strength (Rm) of the cans measured before and after the curing oven, in which the inner varnish layer was polymerized, were evaluated. Moreover, the hardness (HB) of the input semifinished products (slugs) was measured.

**Table 1**

| Alloy | Hardness of the slug | Tensile strength Rm [MPa] | | | |
|---|---|---|---|---|---|
| | | After the backward extrusion | After the curing (polymerization) oven of inner varnish | | |
| | | | 210°C/10min | 230°C/10min | 255°C/10min |
| A5 | 20.8 | 164.1 | 154.8 | 150.5 | 135.1 |
| A3Mn | 22 | 180.7 | 172.6 | 167.9 | 151.2 |
| MC1_A | 22 | 171.0 | 171.1 | 168.3 | 167.2 |
| MC3_A | 23.5 | 182.5 | 179.2 | 179.0 | 178.3 |

The results listed in Table 1 clearly show that the standard materials lose their tensile strength when being subject to the temperature of 255°C in the oven, the strength being decreased by 17.7% for aluminium A5 and by 16.3% for the alloy A3Mn. In contrast to that, the loss of strength of the alloys containing Zr is significantly lower, namely only 2.2% for the alloy MC1_A and 2.3% for the alloy MC3_A. In several cases, even an increase of the tensile strength of the new alloys was observed after they had passed through the curing oven.

The comparison of aluminium A5 with the alloy MC1_A shows that the value of the tensile strength of the latter alloy was by 32.1 MPa higher after the passage through the polymerization oven under the temperature of 255°C.

The comparison of aluminium alloys A3Mn and MC3_A shows that the value of the tensile strength of the latter alloy was by 27.1 MPa higher after the passage through the polymerization oven under the temperature of 255°C.

Also advantageous proves to be the fact that although the alloy MC1_A containing the added Zr constituent has its tensile strength after the backward extrusion by 9.7 MPa lower in comparison with the alloy A3Mn, the passage of the alloy MC1_A through the polymerization oven under temperatures over 226°C causes the strength of this alloy to exceed the strength of the A3Mn alloy, even though the MC1_A alloy does not contain Mn.

The main advantages of the new alloys MC1, MC3 and MC4 particularly include:
a.) Owing to the admixture of Zr, the alloys MC1, MC3 and MC4 contain a fine dispersion of Al₃Zr.
b.) The presence of manganese in the alloys MC3 and MC4 additionally results in an increase of the strength of these alloys after undergoing a shaping process, this being due to the formation of the particles of Al₆Mn, Al₆(FeMn) and α-Al(Mn,Fe)Si.
c.) The above particles become caught in the subgrain boundaries, thus preventing any recovery, formation of recrystallization nuclei or growth of recrystallized grains from occurring (increasing the recrystallization resistance).

## Claims

1. Heat-resistant alloy for production of aerosol cans from a material having the following contents of alloying additions in percent by weight:
according to the standards EN 573-3
EN AW 3207
Si ≤ 0.30; Fe ≤ 0.45; Cu ≤ 0.10; Mn 0.40-0.80; Mg ≤ 0.10; Zn ≤ 0.10;
or with more specific compositions
- Si = 0.05÷0.09; Fe = 0.23÷0.27; Cu ≤ 0.005; Mn = 0.58÷0.62; Mg ≤ 0.005; Zn ≤ 0.015; Ti = 0.01÷0.03;
**characterized in that** each composition contains added Zr in the amount ranging between 0.10 and 0.15% by weight, the sum of the contained amounts of all the secondary elements being ≤ 0,10% by weight and Al content is remainder.

## Patentansprüche

1. Warmbeständige Legierung für Produktion von Aerosolkontainer aus dem Material mit Zusätzeninhalt in Gewicht %:
nach der EN 573-3 Norm:
EN AW 3207
Si ≤ 0.30; Fe ≤ 0.45; Cu ≤ 0.10; Mn 0.40-0.80; Mg ≤ 0.10; Zn ≤ 0.10;
oder bei einem präzisierten Zusammensetzung von
Si = 0.05÷0.09; Fe = 0.23÷0.27; Cu ≤ 0.005; Mn = 0.58÷0.62; Mg ≤ 0.005; Zn ≤ 0.015; Ti = 0.01÷0.03;
**dadurch gekennzeichnet, dass** die Komposition Zr im Bereich von 0,10 bis 0,15% Gewicht % beinhaltet und dsie Summe von allen Beielementen ist ≤ 0,10 und der Aluminiumgehalt ist der Rest.

## Revendications

1. Un alliage thermo-résistant, destiné a la production de récipiente a l'aérosol de composition chemique suivante:
apres la norme EN 573-3
EN AW 3207
Si ≤ 0.30; Fe ≤ 0.45; Cu ≤ 0.10; Mn 0.40-0.80; Mg ≤ 0.10; Zn ≤ 0.10;
ou plus précisement
Si = 0.05÷0.09; Fe = 0.23÷0.27; Cu ≤ 0.005; Mn = 0.58÷0.62; Mg ≤ 0.005; Zn ≤ 0.015; Ti = 0.01÷0.03;
**caractérisé, en ce que** chaque composition comporte Zr entre 0,10-0,15% et les autres inoculants ≤ 0,10% . Le reste de l'alliage est fait par l'aluminium.
